

[54] **FOGGED, DIRECT-POSITIVE SILVER HALIDE EMULSION OPTICALLY SENSITIZED WITH A DYE CONTAINING A PYRROLO[2,1-B]THIAZOLE NUCLEUS.**

[75] Inventors: **Henri Depoorter, Mortsel; Felix Jan Moelants, Wilrijk, both of Belgium**

[73] Assignee: **AGFA-GEVAERT N.V., Mortsel, Belgium**

[22] Filed: **Apr. 24, 1974**

[21] Appl. No.: **463,804**

[30] **Foreign Application Priority Data**

Apr. 25, 1973 United Kingdom..... 19616/73

[52] **U.S. Cl.** ..... 96/101; 96/107; 96/108; 96/130; 260/240 E

[51] **Int. Cl.<sup>2</sup>** ..... G03C 1/02; G03C 1/36

[58] **Field of Search** ..... 96/107, 108, 101, 130; 260/240 E

[56] **References Cited**  
UNITED STATES PATENTS

3,772,278 11/1973 Jeffreys et al..... 96/130  
3,809,691 5/1974 Carpenter et al..... 96/101

*Primary Examiner*—Won H. Louie, Jr.  
*Attorney, Agent, or Firm*—A. W. Breiner

[57] **ABSTRACT**

A direct-positive photographic element is described which comprises a support and a spectrally-sensitized light-sensitive silver halide emulsion layer containing fogged silver halide grains wherein the said emulsion is spectrally sensitized by means of a dye containing a pyrrolo[2,1-b]thiazole nucleus which may be substituted and carry one or more fused-on rings, the said nucleus being linked by the 5- or 7-carbon atom thereof, directly or through a dimethine chain to another nitrogen containing heterocycle.

**8 Claims, No Drawings**

FOGGED, DIRECT-POSITIVE SILVER HALIDE  
EMULSION OPTICALLY SENSITIZED WITH A  
DYE CONTAINING A PYRROLO[2,1-B]THIAZOLE  
NUCLEUS

The present invention relates to spectrally sensitized direct positive silver halide emulsions.

It is known that direct-positive images can be obtained with certain types of photographic silver halide emulsions without previously forming a negative silver image. For this purpose, the silver halide grains are fogged by an overall-exposure to actinic radiation or by an overall chemical fogging, e.g. by means of reducing agents, before or after they are coated on a support. Upon image-wise exposure of the pre-fogged emulsions the development centres formed by said fogging are destroyed at the exposed areas and remain at the unexposed areas. By subsequent conventional development by means of silver halide developers a direct-positive image is formed.

For the spectral sensitization of negative-type silver halide emulsions there is a wide choice of spectrally sensitizing dyes such as mono- and trimethine cyanines, rhodacyanines, hemicyanines, merocyanines, styryl dyes, oxonol dyes, etc. Most of these dyes, however, are unsuitable for the spectral sensitization of direct-positive emulsions.

The choice of really suitable sensitizing dyes for direct-positive emulsions is rather poor and therefore novel spectrally sensitizing dyes for direct-positive emulsions are still needed and sought after.

In accordance with the present invention dyes are provided, which are particularly suitable for the spectral sensitization of direct-positive silver halide emulsions comprising fogged silver halide grains.

The present invention thus provides a direct-positive photographic silver halide element comprising at least one spectrally sensitized direct-positive silver halide emulsion wherein the said emulsion comprises a spectrally sensitizing dye containing a pyrrolo[2,1-b]thiazole nucleus including a substituted pyrrolo[2,1-b]thiazole nucleus and a pyrrolo[2,1-b]thiazole nucleus with one or more fused-on rings e.g. benzo rings, the said nucleus being linked by the 5- or 7-carbon atom thereof, directly or through a dimethine chain, to another nitrogen-containing heterocycle.

The spectrally sensitizing dyes for use according to the present invention can be represented by the following general formula I:



wherein:

Q represents a pyrrolo[2,1-b]thiazol-5- or -7-yl nucleus, which may be substituted and/or carry one or more fused-on rings e.g. benzo rings, more particularly a pyrrolo[2,1-b]thiazolyl group of the formula:



wherein:

each of R<sub>1</sub>, R<sub>2</sub>, R<sub>3</sub> and R<sub>4</sub> represents hydrogen or a substituent e.g. alkyl including substituted alkyl or aryl including substituted aryl, or R<sub>1</sub> together with R<sub>2</sub> and/or R<sub>3</sub> together with R<sub>4</sub> represent the atoms necessary to complete a fused-on 5- or 6-membered ring,

each of L<sub>1</sub>, L<sub>2</sub>, L<sub>3</sub> and L<sub>4</sub> represents a methine group or substituted methine group,

each of m and n represent 0 or 1,

R<sub>5</sub> represents a substituent of the type contained in cyanine dyes on the cyanine nitrogen atom, for example an aliphatic group including a saturated aliphatic group, an unsaturated aliphatic group and a cycloaliphatic group e.g. alkyl, aralkyl, allyl and cycloalkyl or an aromatic group, which groups may carry substituents; more particularly an alkyl group such as methyl, ethyl, propyl, isopropyl, butyl or isobutyl, a substituted alkyl group such as  $\beta$ -hydroxyethyl,  $\beta$ -acetoxethyl, carboxymethyl, carboxyethyl, sulphoethyl, sulphopropyl, sulphobutyl, sulphatopropyl, sulphatobutyl, phosphonoethyl, phosphonopropyl, phosphonobutyl, the group  $-A-CO-O-B-SO_2-OH$  wherein A and B have the same significance as set forth in United Kingdom Patent Specification No. 886,271 such as sulphocarbomethoxymethyl,  $\omega$ -sulphocarbopropoxymethyl,  $\omega$ -sulphocarbobutoxymethyl, and p-( $\omega$ -sulphocarbobutoxy)-benzyl, the group  $-A-W-NH-V-B$  as described in United Kingdom Patent Specification No. 904,332 wherein each of W and V represents carbonyl, sulphonyl or a single bond, at least one of W and V being sulphonyl, A represents an alkylene group e.g. a C<sub>1</sub>-C<sub>4</sub> alkylene group and B represents hydrogen, alkyl, substituted alkyl, amino, substituted amino e.g. acylamino, diethylamino with the proviso however that B does not represent hydrogen when V stands for carbonyl or sulphonyl, the group AWNHVB being exemplified by N-(methylsulphonyl)-carbamylmethyl,  $\gamma$ -(acetylsulphonyl)propyl, and  $\delta$ -(acetylsulphonyl)-butyl, an aralkyl group such as a benzyl, a substituted aralkyl group such as carboxybenzyl and sulphobenzyl, a cycloalkyl group such as cyclohexyl, an allyl group, an aryl group such as phenyl, and a substituted aryl group such as carboxyphenyl,

X<sup>-</sup> stands for an anion of the type contained in cyanine dye salts such as halide, perchlorate, methyl sulphate, benzene sulphonate, p-toluene sulphonate, etc. but does not exist when the molecule itself e.g. R<sub>5</sub> contains an anionic group in which case the dye is a betaine dye salt, and

Z stands for the non-metallic atoms necessary to complete a 5- or 6-membered heterocyclic nucleus containing nitrogen, which nucleus may carry a fused-on benzene or naphthalene ring and further substituents; these heterocycles are of the type known in cyanine dye chemistry and include those of the thiazole series, e.g. thiazole, 4-methylthiazole, 4-phenylthiazole, 5-methylthiazole, 5-phenylthiazole, 4,5-dimethylthiazole, 4,5-diphenylthiazole, 4-(2-thienyl)thiazole, those of the benzothiazole series, e.g. benzothiazole, 5-chlorobenzothiazole, 5-methylbenzothiazole, 6-methylbenzothiazole, 5,6-dimethylbenzothiazole, 5-bromoben-

zothiazole, 5-iodobenzothiazole, 5-phenylbenzothiazole, 5-methoxybenzothiazole, 6-methoxybenzothiazole, 4,5,6,7-tetrahydrobenzothiazole, 5,6-dimethoxybenzothiazole, 5,6-dioxymethylenebenzothiazole, 5-hydroxybenzothiazole, 6-hydroxybenzothiazole, 5-carboxybenzothiazole, 5-sulphobenzothiazole, 5-ethoxycarbonyl benzothiazole, 5-acetylbenzothiazole, 5-benzoylbenzothiazole, 5-cyanobenzothiazole, 5-trifluoromethylbenzothiazole, 6-nitrobenzothiazole, 5-methylsulphonylbenzothiazole, 5-trifluoromethylsulphonylbenzothiazole, those of the naphthothiazole series e.g. naphtho[2,1-d]thiazole, naphtho[1,2-d]thiazole, 5-methoxy naphtho[1,2-d]thiazole, 5-ethoxynaphtho[1,2-d]thiazole, 8-methoxynaphtho[2,1-d]thiazole, 7-methoxynaphtho[2,1-d]thiazole, those of the thionaphtheno[7,6-d]thiazole series e.g. 7-methoxy-thionaphtheno[7,6-d]thiazole, those of the oxazole series e.g. 4-methyloxazole, 5-methyloxazole, 4-phenyloxazole, 4,5-diphenyloxazole, 4-ethyloxazole, 4,5-dimethyloxazole, 5-phenyloxazole, those of the benzoxazole series e.g. benzoxazole, 5-chlorobenzoxazole, 5-methylbenzoxazole, 5-phenylbenzoxazole, 6-methylbenzoxazole, 5,6-dimethylbenzoxazole, 5-methoxybenzoxazole, 6-methoxybenzoxazole, 5-hydroxybenzoxazole, 6-hydroxybenzoxazole, 5-sulphamylbenzoxazole, 5-benzoylbenzoxazole, 5-sulphobenzoxazole, 5-carboxybenzoxazole, 5-β-carboxyvinylbenzoxazole, 5-ethoxycarbonyl benzoxazole, 5-benzoyl-benzoxazole, 6-methoxycarbonylbenzoxazole, those of the naphthoxazole series, e.g. naphtho[2,1-d]oxazole, naphtho[1,2-d]oxazole, those of the selenazole series e.g. 4-methylselenazole, 4-phenylselenazole, those of the benzoselenazole series e.g. benzoselenazole, 5-chlorobenzoselenazole, 5-methylbenzoselenazole, 5,6-dimethylbenzoselenazole, 5-methoxybenzoselenazole, 5-methyl-6-methoxybenzoselenazole, 5,6-dioxymethylenebenzoselenazole, 5-hydroxybenzoselenazole, 4,5,6,7-tetrahydrobenzoselenazole, those of the naphthoselenazole series e.g. naphtho[2,1-d]selenazole, naphtho[1,2-d]selenazole, those of the thiazoline series e.g. thiazoline, 4-methylthiazoline, 4-hydroxymethyl-4-methylthiazoline, 4,6-bis-hydroxymethylthiazoline, those of the oxazoline series e.g. oxazoline, those of the selenazoline series e.g. selenazoline, those of the 2-quinoline series, e.g. quinoline, 6-methylquinoline, 6-chloroquinoline, 6-methoxyquinoline, 6-ethoxyquinoline, 6-hydroxyquinoline, those of the 4-quinoline series e.g. quinoline, 6-methoxyquinoline, 7-methylquinoline, 8-methylquinoline, those of the 1-isoquinoline series, e.g. isoquinoline, 3,4-dihydroisoquinoline, those of the 3-isoquinoline series e.g. isoquinoline, those of the 2-pyridine series e.g. pyridine, 5-methylpyridine, those of the 3,3-dialkyldolenine series e.g. 3,3-dimethylindolenine, 3,3-dimethyl-5-chloroindolenine, 3,3-dimethyl-5 or 6-nitroindolenine, 3,3-dimethyl-5 or 6-cyanoindolenine, 3,3,5-trimethylindolenine, 3,3,7-trimethylindolenine, 3,3-dimethyl-5-ethoxycarbonylindolenine, 3,3-dimethyl-5-carboxyindolenine, 3,3-dimethyl-5-methylsulfonylindolenine, those of the benzimidazole series e.g. benzimidazole, 5,6-dichlorobenzimidazole, 5-chlorobenzimidazole, 5,6-dibromobenzimidazole, 5-phenylbenzimidazole, 5-fluorobenzimidazole,

5,6-difluorobenzimidazole, 5-cyanobenzimidazole, 5,6-dicyanobenzimidazole, 5-chloro-6-cyanobenzimidazole, 5-fluoro-6-cyanobenzimidazole, 5-acetylbenzimidazole, 5-carboxybenzimidazole, 5-ethoxycarbonylbenzimidazole, 5-sulphamylbenzimidazole, 5-N-ethylsulphamylbenzimidazole, 5-ethylsulphonylbenzimidazole and 5-trifluoromethylsulphonylbenzimidazole, etc.

A preferred class of spectrally sensitizing dyes for use according to the present invention in direct-positive silver halide emulsions can be represented by the following general formula II:



wherein:

Q, L<sub>1</sub>, L<sub>2</sub>, L<sub>3</sub>, L<sub>4</sub>, m, n, R<sub>5</sub> and X have one of the significances given above,

Y represents the atoms necessary to close a fused-on benzo or naphtho ring carrying one or more substituents at least one of which is a substituent with a Hammett constant  $\sigma\rho$  of at least 0.30 for example a nitro group, a cyano group, a carboxyl or sulpho group, an alkoxy carbonyl group such as methoxycarbonyl a carboxylic acyl group e.g. acetyl and benzoyl, a trifluoromethyl group, a cyanovinyl group, a fluorosulphonyl group, an alkylsulphonyl group e.g. methylsulphonyl including a substituted alkylsulphonyl group such as alkylsulphonyl wherein the alkyl group is substituted by one or more fluorine and/or chlorine atoms, an alkylsulphanyl group or substituted alkylsulphanyl group such as alkylsulphanyl wherein the alkyl group is substituted by one or more fluorine and/or chlorine atoms, a trifluoromethoxy group, a trifluoromethylthio group, a difluoromethylthio group, a carbamoyl group



or sulphamoyl group



wherein each of R<sub>7</sub> and R<sub>8</sub>, the same or different, stands for hydrogen or a saturated or unsaturated aliphatic group including a substituted aliphatic group such as alkyl, preferably C<sub>1</sub>-C<sub>5</sub> alkyl, cycloalkyl, e.g. cyclohexyl, or allyl, or R<sub>7</sub> together with R<sub>8</sub> represent the atoms necessary to close a heterocyclic ring such as pyrrolidine, piperidine, piperazine and morpholine, a  $-\text{SO}_2\text{NCO}$  alkyl group, etc., and

Z<sub>1</sub> when n is 0, stands for oxygen, sulphur, selenium,

alkyl  
C  
alkyl  
or  $L_5=L_6$  wherein  $L_5$  and  $L_6$  represent methine or

substituted methine, and when  $n$  is 1, stands for a monovalent chemical bond.

Representative examples of spectrally sensitizing dyes suitable for use in accordance with the present invention are listed in the table hereinafter.

Table

| Dye | Structural formula                                                                  | Absorp-<br>tion<br>maxi-<br>mum<br>nm | Extinc-<br>tion<br>coeffi-<br>cient<br>$\times 10^{-5}$ |
|-----|-------------------------------------------------------------------------------------|---------------------------------------|---------------------------------------------------------|
| 1.  |    | 522                                   | 1.0                                                     |
| 2.  |    | 557                                   | 1.1                                                     |
| 3.  |  | 559                                   | 1.2                                                     |
| 4.  |  | 558                                   | 1.3                                                     |
| 5.  |  | 555                                   | 1.3                                                     |
| 6.  |  | 562                                   | 1.3                                                     |

Table

| Dye | Structural formula | Absorp-<br>tion<br>maxi-<br>mum<br>nm | Extinc-<br>tion<br>coeffi-<br>cient<br>$\times 10^{-5}$ |
|-----|--------------------|---------------------------------------|---------------------------------------------------------|
| 7.  |                    | 513                                   | 0.87                                                    |
| 8.  |                    | 516                                   | 0.82                                                    |
| 9.  |                    | 522                                   | 1.0                                                     |
| 10. |                    | 520                                   | 0.97                                                    |
| 11. |                    | 523                                   | 0.78                                                    |
| 12. |                    | 554                                   | 0.72                                                    |

Table

| Dye | Structural formula | Absorp-<br>tion<br>maxi-<br>mum<br>nm | Extinc-<br>tion<br>coeffi-<br>cient<br>$\times 10^{-5}$ |
|-----|--------------------|---------------------------------------|---------------------------------------------------------|
| 13. |                    | 556                                   | 0.72                                                    |
| 14. |                    | 558                                   | 0.93                                                    |
| 15. |                    | 548                                   | 0.71                                                    |
| 16. |                    | 554                                   | 0.81                                                    |
| 17. |                    | 561                                   | 0.79                                                    |
| 18. |                    | 560                                   | 0.81                                                    |

Table

| Dye | Structural formula | Absorp-<br>tion<br>maxi-<br>mum<br>nm | Extinc-<br>tion<br>coeffi-<br>cient<br>$\times 10^5$ |
|-----|--------------------|---------------------------------------|------------------------------------------------------|
| 19. |                    | 555                                   | 0.91                                                 |
| 20  |                    | 559                                   | 0.85                                                 |
| 21  |                    | 550                                   | 1.1                                                  |
| 22  |                    | 566                                   | 0.93                                                 |
| 23  |                    | 525                                   | 0.97                                                 |

Table

| Dye | Structural formula | Absorp-<br>tion<br>maxi-<br>mum<br>nm | Extinc-<br>tion<br>coeffi-<br>cient<br>$\times 10^{-5}$ |
|-----|--------------------|---------------------------------------|---------------------------------------------------------|
| 24  |                    | 552                                   | 0.69                                                    |
| 25  |                    | 589                                   | 0.57                                                    |
| 26  |                    | 558                                   | 1.02                                                    |
| 27  |                    | 556                                   | 1.23                                                    |
| 28  |                    | 520                                   | 0.97                                                    |
| 29  |                    | 550                                   | 0.95                                                    |

15  
-continued

## 16

Table

| Dye | Structural formula | Absorp-<br>tion<br>maxi-<br>mum<br>nm | Extinc-<br>tion<br>coeffi-<br>cient<br>$\times 10^5$ |
|-----|--------------------|---------------------------------------|------------------------------------------------------|
| 30  |                    |                                       |                                                      |
| 31  |                    | 551                                   | 0.68                                                 |
| 32  |                    | 562                                   | 0.82                                                 |
| 33  |                    | 560                                   | 0.94                                                 |
| 34  |                    | 559                                   | 1.02                                                 |
| 35  |                    | 530                                   | 0.58                                                 |
|     |                    | 564                                   | 0.74                                                 |

Table

| Dye | Structural formula | Absorp-<br>tion<br>maxi-<br>mum<br>nm | Extinc-<br>tion<br>coeffi-<br>cient<br>$\times 10^5$ |
|-----|--------------------|---------------------------------------|------------------------------------------------------|
| 36  |                    | 562                                   | 0.57                                                 |
| 37  |                    | 540                                   | 0.48                                                 |
| 38  |                    | 562                                   | .01                                                  |
| 39  |                    | 519                                   | 0.91                                                 |
| 40  |                    |                                       |                                                      |

Table

| Dye | Structural formula | Absorp-<br>tion<br>maxi-<br>mum<br>nm | Extinc-<br>tion<br>coeffi-<br>cient<br>$\times 10^{-5}$ |
|-----|--------------------|---------------------------------------|---------------------------------------------------------|
| 41  |                    | 559<br>521                            | 1.3<br>0.75                                             |
| 42  |                    | 522                                   | 0.84                                                    |
| 43  |                    | 553                                   | 0.99                                                    |
| 44  |                    | 569                                   | 0.92                                                    |
| 45  |                    | 565                                   | 0.68                                                    |
| 46  |                    | 552                                   | 0.68                                                    |

Table

| Dye | Structural formula | Absorp-<br>tion<br>maxi-<br>mum<br>nm | Extinc-<br>tion<br>coeffi-<br>cient<br>$\epsilon \times 10^{-5}$ |
|-----|--------------------|---------------------------------------|------------------------------------------------------------------|
| 47  |                    | 559                                   | 0.11                                                             |
| 48  |                    | 551                                   | 0.84                                                             |
| 49  |                    | 547                                   | 1.3                                                              |
| 50  |                    | 542                                   | 1.0                                                              |
| 51  |                    | 533                                   | 0.86                                                             |

The dyes for use in accordance with the present invention can be prepared according to methods described by S. Mc Kenzie et al., in J. Chem. Soc. C (1966) 1908; F. S. Babichev et al. in Ukr. Khim. Zhurn. 32 (1966) 64; F. S. Babichev et al. in J. Gen. Chem. USSR 33 (1963) 1946 — 33 (1963) 3518.

For example, the dimethine dyes can be prepared, as is illustrated by the preparations hereinafter by condensing, preferably in the presence of an acid anhydride e.g. acetic anhydride, a compound of the following formula III:



55 wherein:

$\text{L}_3-\text{L}_4$ ,  $\text{Z}$ ,  $\text{R}_5$ ,  $\text{X}$  and  $n$  have the same meaning as above, with a pyrrolo[2,1-b]thiazole-5- or 7-carboxaldehyde of the following formula IV:

60 IV.  $\text{Q}-\text{CH}=\text{O}$

wherein:

$\text{Q}$  has the same meaning as above.

The intermediates of formula IV can be prepared from the corresponding pyrrolo[2,1-b]thiazole compound by a Vilsmeier and Haack reaction with dimethylformamide as formylating agent.

The dyes of the above general formulae I and II wherein  $m$  is 0 can be prepared by condensation of the

pyrrolo[2,1-b]thiazole unsubstituted in the 5- and/or 7-position with a compound of the following formula V:



wherein:

$\text{L}_3$ ,  $\text{L}_4$ ,  $\text{Z}$ ,  $\text{R}_5$  and  $\text{X}$  have the same meaning as above, and Alk stands for lower alkyl, e.g. methyl.

The following preparations illustrate how the dyes for use according to the invention were prepared.

#### Preparation 1 — Dye 4

A mixture of 3-methyl-5-formyl-6-phenyl-pyrrolo[2,1-b]thiazole (2.41 g; 0.01 mole), 1,2,3,3-tetramethyl-5-ethoxycarbonyldolneniumiodide (3.73 g; 0.01 mole) and acetic anhydride (40 ml) was refluxed for 15 minutes. After cooling, the precipitated dye was filtered off by suction and recrystallized from methanol.

Yield: 4.8 g. Melting point: 180°C.

I%: Calc.: 21.3% Found: 20.9%.

#### Preparation 2 — Dye 6

To 3-methyl-5-formyl-6-phenyl-pyrrolo[2,1-b]thiazole (2.41 g; 0.01 mole) and 1,3,3-trimethyl-2-methylene-5-nitroindoline (2.18 g; 0.01 mole) in acetic anhydride (45 ml), sodium acetate (1.6 g) was added. The mixture was refluxed for 0.5 hours, cooled, filtered and washed with water. The dye was dissolved in boiling methanol, treated with charcoal and converted into the iodide by adding 3 g of sodium iodide.

Yield: 200 g. Melting point: above 260°C.

I%: Calc.: 22.3% Found: 21.7%.

#### Preparation 3 — Dye 9

A mixture of 3-methyl-5-formyl-6-phenyl-pyrrolo[2,1-b]thiazole (2.41 g; 0.01 mole), 2-methyl-3-ethyl-5-phenylbenzoxazolium iodide (3.65 g; 0.01 mole) and acetic anhydride was refluxed for 10 minutes. After cooling, the mixture was poured into ether (300 ml) and the precipitated dye recrystallized from 2-methoxyethanol.

Yield: 2.8 g. Melting point: above 260°C.

I%: Calc.: 21.6% Found: 21.2%.

#### Preparation 4 — Dye 24

3-methyl-5-formyl-6-phenylpyrrolo[2,1-b]thiazole (2.41 g; 0.01 mole), 1-methyl-chinaldinium methylsulphate (2.69 g; 0.01 mole) and acetic anhydride (45 ml) was refluxed for 5 minutes. After cooling, the crude dye was collected by filtration, washed with ether and treated with charcoal in boiling methylene chloride. The solution was filtered and the filtrate was poured into ether and the precipitate was chromatographed in methylene chloride on alumina (elution by methylene chloride containing 1% methanol).

Yield: 1.0 g. Melting point: 180°C (decomp.).

I%: Calc.: 13.0% Found: 12.8%.

#### Preparation 5 — Dye 29

A mixture of 3-methyl-5-formyl-6-(4-bromophenyl)-pyrrolo[2,1-b]thiazole (3.2 g; 0.01 mole), 2,3-trimethyl-5-trifluoromethylbenzothiazolium p-tolusulphonate (4.03 g, 0.01 mole) and acetic anhydride (40 ml) was

boiled for 10 minutes, cooled and filtered with suction. As shown by T.L.C. the dye was obtained in pure state.

Yield: 5.5 g. Melting point: 150°C (decomp.).

I%: Calc.: 8.08% Found: 8.10%.

#### Preparation 6 — Dye 35

3-methyl-5-formyl-6-(4-nitrophenyl)pyrrolo[2,1-b]thiazole (1.43 g; 0.005 mole), 2-methyl-3-ethyl-5-methylsulphonylbenzothiazolium ethylsulphate (1.9 g; 0.005 mole) and acetic anhydride (25 ml) were refluxed for 5 minutes. The dye formed was collected by filtration, washed with ether and digested with 300 ml of boiling methanol.

Yield: 2.5 g. Melting point: above 360°C.

I%: Calc.: 19.7% Found: 19.8%.

The methods of incorporating the dyes in the emulsions are relatively simple and well known to those skilled in the art of emulsion making.

The dyes according to the present invention are usually added to the direct-positive silver halide emulsion in the form of a solution in a suitable solvent, e.g. water, lower alcohols such as methanol and ethanol, ketones such as acetone, amines such as triethylamine, pyridine, mixtures of these solvents and other well-known solvents known in the art. The dyes may be used in widely varying concentrations. They are generally used in amounts varying from about 50 mg to about 2 g per mole of silver halide. The optimum concentration is dependent on the particular dye concerned and the particular emulsion used and can be determined readily by methods known to those skilled in the art.

The direct-positive silver halide emulsions can be prepared according to known methods. The silver halide composition may consist of any of the known silver halides suitable for the formation of direct-positive silver halide emulsions e.g. silver bromide, silver chloride, silver chlorobromide, silver bromoiodide and silver chlorobromoiodide. Emulsion blends can also be used e.g. blends of silver chloride and silver chlorobromide. The silver halide preferably comprises at most 20 mole % of silver iodide which may be located mainly towards the surface of the grains as described in German Patent Application No. P 22 60 117.8.

Especially suitable for use according to the present invention are direct-positive silver halide emulsions the silver halide grains of which have an average grain-size of less than about 1 micron. The silver halide grains can be regular and have one of the commonly known shapes e.g. cubic, octahedral, and even rhombohedral.

They may have a substantially uniform diameter frequency distribution e.g. 95% by weight of the silver halide grains can have a diameter which is within about 40%, preferably within about 30% of the mean grain diameter.

The silver halide grains of the direct-positive silver halide emulsions of the present invention are fogged according to methods well known in the art. They may be fogged e.g. by an overall exposure to actinic radiation or by reduction sensitization e.g. by high pH and/or low pAg silver halide precipitating or digestion conditions e.g. as described by Wood, J. Phot. Sci. 1 (1953) 163, or by treatment with reducing agents. Fogging may also occur by reduction sensitization in the presence of a compound of a metal more electro-positive than silver.

Reducing agents suitable for use include hydrazine, hydroxylamine, tin(II) compounds e.g. tin(II) chloride, tin complexes and tin chelates of the (poly)amino(-

poly)carboxylic acid type as described in United Kingdom Patent No. 1,209,050, ascorbic acid, formaldehyde, thiourea dioxide, polyamines such as diethylene triamine, phosphonium salts such as tetra(hydroxymethyl)phosphonium chloride, bis(p-aminoethyl) sulphide and its water-soluble salts, etc. Preferred reducing agents are thiourea dioxide and tin(II) chloride.

The compounds of a metal more electropositive than silver include gold compounds e.g. gold(III)chloride, potassium chloroaurate, potassium chloroaurite, and potassium aurithiocyanate, as well as compounds of rhodium, platinum, iridium and palladium, e.g. ammonium hexachloropalladate and potassium chloroiridate. Preferred noble metal compounds are gold compounds.

When fogging of the silver halide grains occurs by means of a reducing agent e.g. thiourea dioxide and a compound of a metal more electropositive than silver especially a gold compound, the reducing agent is preferably used initially and the gold compound subsequently. However, the reverse order can be used or both compounds can be used simultaneously.

The degree of fogging of the direct-positive emulsions used according to the invention may vary within a wide range. This degree of fogging depends, as is known in the art, on the concentration of the fogging agents used as well as on the pH, the pAg, the temperature and the duration of the fogging treatment.

As is known in the art, high photographic speeds can be obtained at low degrees of fogging. Thus, the direct-positive silver halide emulsions of the invention can be fogged, as is described in U.S. Pat. No. 3,501,307, to such a degree that a test-portion of the silver halide emulsion, comprising the fogged silver halide grains and a compound accepting electrons, when coated on a support to give a maximum density of at least about one upon processing for 6 minutes at about 20°C in a developer of the composition given below, has a maximum density which is at least about 30% greater than the maximum density of an identical test portion processed for 6 minutes at about 20°C in the same developer after being bleached for about 10 minutes at about 20°C in a bleach of the composition given below:

|                                 |         |
|---------------------------------|---------|
| <u>bleach :</u>                 |         |
| potassium cyanide               | 50 mg   |
| glacial acetic acid             | 3.47 ml |
| sodium acetate                  | 11.49 g |
| potassium bromide               | 119 mg  |
| water to make                   | 1 liter |
| <u>developer :</u>              |         |
| N-methyl-p-aminophenol sulphate | 2.5 g   |
| sodium sulphite                 | 30.0 g  |
| hydroquinone                    | 2.5 g   |
| sodium metaborate               | 10.0 g  |
| potassium bromide               | 0.5 g   |
| water to make                   | 1 liter |

In order to further enhance the photographic speed, the silver halide grains of the direct-positive silver halide grains of the present invention may be fogged even to a degree where strictly speaking no fogging as defined in the said U.S. Pat. No. 3,501,307 is observed, e.g. as described in co-pending United Kingdom Patent Application No. 7742/72. According to this co-pending application the silver halide grains are fogged to such an extent that a test portion of the emulsion ready for coating, when coated on a support at a coverage of 0.50 g to 5.50 g of silver per sq.m gives a density of less than 0.50 upon processing without exposure for 6 min.

at 20°C in the above developer and an identical test portion thereof when coated in an identical way gives a density of at least twice the value of the density of the first test portion and a density of at least 0.50 upon processing without exposure for 3 minutes at 20°C in a developer of the following composition:

|                                                     |         |
|-----------------------------------------------------|---------|
| hydroquinone                                        | 15 g    |
| 1-phenyl-3-pyrazolidinone                           | 1 g     |
| trisodium salt of ethylene diamine tetraacetic acid | 1 g     |
| anhydrous sodium carbonate                          | 30 g    |
| anhydrous sodium sulphite                           | 70 g    |
| 40% aqueous sodium hydroxide                        | 16 ml   |
| water to make                                       | 1 liter |

(pH : 11)

15

When the silver halide grains have been fogged too heavily it is also possible to treat the fogged silver halide grains with a bleaching agent in order to obtain optimum sensitivity.

In view of the foregoing, the terms "fogged" and "fogging" as used herein are employed in a very broad sense so that the very low degrees of fogging as defined in the above copending United Kingdom Patent Application are also embraced which means that fogging is effected to such extent that a test portion of the emulsion when coated as described above gives a density of at least 0.50 upon processing for 3 min. at 20°C in the above latter developer composition.

When the silver halide grains are fogged to a very low degree it is advantageous to develop the exposed direct-positive silver halide emulsions substantially in the absence of halide ions as described in United Kingdom Patent Application No. 7743/72.

The speed and stability of the direct-positive silver halide emulsions according to the present invention can also be enhanced by increasing the pAg of the emulsion just before coating, preferably after addition of the spectral sensitizer. Favourable photographic speeds are obtained when the pAg is adjusted, before coating, to a value corresponding to an E.M.F. of +30 mV or lower (silver against saturated calomel electrode). It is also favourable to further enhance the speed to lower the pH of the emulsion just before coating for example to a pH of at least about 5 as described in United Kingdom Patent Application No. 32889/72.

In the formation of the direct-positive silver halide emulsions used according to the present invention various colloids can be used as vehicles or binding agents for the silver halide. They include any of the hydrophilic colloids generally employed in the photographic field for example gelatin. However, the gelatin may be replaced wholly or partly by other natural hydrophilic colloids, e.g. albumin, zein, agar-agar, gum arabic, alginic acid, and derivatives thereof, such as esters, amides and salts thereof etc., or synthetic hydrophilic resins; e.g. polyvinyl alcohol and poly-N-vinyl pyrrolidone, acrylamide polymers, cellulose ethers, partially hydrolyzed cellulose acetate and the like.

In addition to the hydrophilic binding agents other synthetic binding agents can be employed in the emulsion e.g. homo- and copolymers of acrylic or methacrylic acid or derivatives thereof such as esters, amides and nitriles and vinyl polymers for example vinyl esters and vinyl ethers.

The direct-positive photographic silver halide emulsions can be coated on a wide variety of supports which include opaque supports e.g. paper and metal supports

as well as transparent supports e.g. glass, cellulose nitrate film, cellulose acetate film, cellulose aceto-butyrate film, polyvinyl acetal film, polystyrene film, polyethylene terephthalate film, polycarbonate film, and other polyester film. It is also possible to employ paper coated with  $\alpha$ -olefin polymers e.g. paper coated with polyethylene, polypropylene, ethylene-butylene copolymers and the like.

The direct-positive emulsions sensitized with dyes according to the present invention may further contain dyes of the type which in silver halide emulsions of the negative type act as desensitizers and therefore are called desensitizing dyes. Particularly suitable for this purpose are the nitrobenzylidene and nitrostyryl dyes described in U.S. Pat. No. 3,615,610. The emulsions may also comprise desensitizing dihydropyrimidine compounds of the type described in U.S. patent application Ser. No. 269,861 (= published German Patent Application No. 2,237,036) as well as other desensitizing compounds e.g. 2,3,5-triphenyl-2H-tetrazolium chloride, 2-(4-iodophenyl)-3-(4-nitrophenyl)-5-phenyl tetrazolium chloride, 1-methyl-8-nitroquinolinium methyl sulphate, 1-m-nitrobenzyl-quinolinium chloride, 1-m-nitrobenzylpyridinium chloride, 1-p-nitrobenzylisoquinolinium chloride, 1-p-nitrobenzylbenzo[f]quinolinium chloride and 1-methyl-2-m-nitrostyrylquinolinium methyl sulphate.

The silver halide emulsion may further contain any of the ingredients generally employed in silver halide emulsions. They may comprise speed increasing agents of the polyalkylene oxide type e.g. polyethylene glycols and derivatives thereof, quaternary ammonium and phosphonium compounds as well as ternary sulphonium compounds, thioether compounds, etc. The emulsions can comprise the common emulsion stabilizing agents, e.g. mercury compounds which include homopolar or salt-like compounds of mercury and aromatic or heterocyclic compounds such as mercaptotriazoles, simple mercury salts, sulphonium mercury double salts, etc. They may comprise azaindene emulsion stabilizers for example tetra- or pentaazaindenes especially those comprising hydroxyl or amino groups as described by Birr, Z. Wiss. Phot. 47 (1962) 2-58. Other suitable emulsion stabilizers are heterocyclic mercapto compounds e.g. 1-phenyl-5-mercaptopentrazole, quaternary benzthiazolium derivatives, benztriazole and the like.

The emulsions may further contain colour forming couplers. Among the useful colour forming couplers are the monomeric and polymeric colour couplers e.g. pyrazolone colour couplers as well as phenolic, heterocyclic and open chain colour couplers having a reactive methylene group.

Particularly suitable are colour couplers showing a low halogen accepting character which can be determined by the test described by R. P. Held in Phot. Sci. Eng. Vol. 11, (1967) p. 406. For this purpose a dispersion of silver bromide grains is buffered 0.1 N potassium bromide is illuminated and the potential is registered by means of a calomel/platinum electrode system. During illumination the platinum electrode potential rises rapidly to the redox potential of bromine. On addition of a colour coupler the potential rise can be delayed through "halogen acceptance" by the colour coupler. Colour couplers that do not delay or do not substantially delay the potential rise are particularly suitable for use in the direct-positive silver halide emulsions of the invention.

The colour couplers can be incorporated into the direct-positive photographic silver halide emulsion according to any suitable technique known to those skilled in the art for incorporating colour couplers in silver halide emulsions. For example, water-soluble colour couplers, e.g. those containing one or more sulpho or carboxyl groups (in acid or salt form), can be incorporated from an aqueous solution, if necessary, in the presence of alkali, and the water-insoluble or insufficiently water-soluble colour couplers from a solution in the appropriate water-miscible or water-immiscible high-boiling (oil-former) or low-boiling organic solvents or mixtures of solvents, which solution is dispersed, if necessary in the presence of a surface-active agent, in a hydrophilic colloid composition forming or forming part of the binding agent of the silver halide emulsion; if necessary, the low-boiling solvent is removed afterwards by evaporation.

The silver halide emulsion layer and any other hydrophilic colloid layer, which may be present in a direct-positive photographic material employed in accordance with the present invention, may be hardened by means of organic or inorganic hardeners commonly employed in photographic silver halide elements, e.g. the aldehydes and blocked aldehydes such as formaldehyde, dialdehydes, hydroxyaldehydes, mucochloric and mucobromic acid, acrolein, glyoxal, sulphonyl halides, vinylsulphones, etc.

The direct-positive photographic silver halide elements may further contain antistatic agents, wetting agents as coating aids, e.g. saponin and synthetic surface-active compounds, plasticizers, matting agents, e.g. starch, silica, polymethyl methacrylate, zinc oxide, titanium dioxide, etc., optical brightening agents including stilbene, triazine, oxazole, and coumarin brightening agents, light-absorbing materials and filter dyes, mordanting agents, for anionic compounds, etc.

The following examples illustrate the present invention.

#### EXAMPLE 1

A monodisperse, cubic direct-positive photographic silver bromoiodide emulsion (2.5 mole % of iodide) having an average grain size of about 0.2 micron, was prepared under controlled pH, pAg, and temperature conditions during precipitation of the silver halide. The pH was maintained at about 5.5, the pAg at 8.2 and the temperature at 45°C. After adjustment of the pAg to 10, the emulsion was chill-set, shredded, and washed with cold water.

The emulsion was reduction- and gold-fogged by adjustment of the pAg to 5.3 and the pH to 7, by heating for 90 min. at 60°C and by the addition of 30 mg of chloroaurate per mole of silver halide. Heating was continued for 80 minutes at 60°C whereupon the pAg was adjusted to 8.2 and 35°C.

The emulsion was divided into several aliquot samples of 100 g comprising 0.15 mole of silver halide. To each sample 87.5 mg of Pinacrytol yellow and 87.5 mg of one of the dyes referred to hereinbefore were added. Then the emulsion samples were coated on a subbed support and dried.

The direct-positive elements obtained were exposed in a spectrograph and developed in a conventional developer. Direct-positive spectrograms were obtained. The spectral sensitization maxima are listed in the following table.

| Spectrally sensitizing dye | Sensitization maxima (nm) |
|----------------------------|---------------------------|
| 1                          | 590                       |
| 2                          | 595                       |
| 3                          | 600                       |
| 4                          | 605                       |
| 5                          | 600                       |
| 6                          | 620                       |
| 9                          | 560                       |
| 10                         | 565                       |
| 11                         | 560                       |
| 14                         | 560                       |
| 24                         | 630                       |
| 25                         | 640                       |
| 28                         | 565                       |
| 29                         | 600                       |
| 30                         | 580                       |
| 35                         | 580                       |

## EXAMPLE 2

A washed silver iodobromide emulsion containing 20 per kg 60 g of silver halide (95 mole % of silver bromide and 5 moles % of silver iodide) and chemically fogged with sodium hydroxide (pH = 12) during the precipitation step and subsequent heat-treatment (15 min. at 55°C and 10 min. at 80°C) was divided into 25 several aliquot portions. To each of these portions one of the sensitizing dyes listed in the table below was added in an amount of 60 mg per kg of emulsion. Then the emulsions were coated on a cellulose triacetate support and dried. The materials were exposed in a 30 sensitometer to white light and then developed in a common hydroquinone/p-N-methylaminophenol hemisulphate mixture and fixed. The sensitization maxima obtained with the dyes of the invention are listed in the table below.

Table

| Spectrally sensitizing dye | Sensitization maxima (nm) |
|----------------------------|---------------------------|
| 7                          | 570                       |
| 8                          | 580                       |
| 12                         | 580                       |
| 13                         | 600                       |
| 15                         | 600                       |
| 16                         | 600                       |
| 17                         | 600                       |
| 18                         | 590                       |
| 19                         | 630                       |
| 20                         | 600                       |
| 21                         | 600                       |
| 22                         | 625                       |
| 23                         | 600                       |

## EXAMPLE 3

To samples of a fogged silver halide emulsion as described in example 1 87.5 mg of Pinacrytol yellow and 87.5 mg of one of the dyes referred to in the table hereinafter were added. The emulsion samples were coated on a support and dried.

The direct-positive elements obtained were exposed in a spectrograph and developed in a conventional developer. The spectral sensitization maxima and the total speed obtained are listed in the table hereinafter. The values given for the total speed are relative values; a value of 100 was given to the emulsion to which no spectrally sensitizing dye was added.

| Dye added | Sens. max.<br>nm | Total speed |
|-----------|------------------|-------------|
| none      | —                | 100         |

| Dye added | Sens. max.<br>nm | Total speed |
|-----------|------------------|-------------|
| 5         | 26               | 560         |
|           | 27               | 400         |
|           | 32               | 1100        |
|           | 33               | 800         |
|           | 34               | 560         |
|           | 36               | 400         |
| 10        | 37               | 280         |
|           | 38               | 800         |
|           | 39               | 1100        |
|           | 40               | 280         |
|           | 41               | 280         |
|           | 42               | 200         |
|           | 43               | 140         |
|           | 44               | 1100        |
| 15        | 45               | 400         |
|           | 46               | 280         |
|           | 48               | 560         |
|           | 49               | 400         |
|           | 50               | 1100        |
|           | 51               | 560         |

We claim:

1. A direct-positive photographic element comprising a support and a spectrally-sensitized light-sensitive silver halide emulsion layer containing fogged silver halide grains wherein the said emulsion is spectrally sensitized by means of a dye containing a pyrrolo[2,1-b]thiazole nucleus, the said nucleus being linked by the 5- or 7-carbon atom thereof, directly or through a dimethine chain to another 5- or 6-membered nitrogen containing heterocycle.

2. A direct-positive photographic element according to claim 1 wherein the dye corresponds to the formula:



40 wherein:

Q represents a pyrrolo[2,1-b]thiazol-5-yl or pyrrolo[2,1-b]thiazol-7-yl nucleus, each of L<sub>1</sub>, L<sub>2</sub>, L<sub>3</sub> and L<sub>4</sub> represents a methine group, each of m and n represents 0 or 1,

45 R<sub>5</sub> represents an aliphatic group or an aromatic group,

X<sup>-</sup> represents an anion but is not present when the balance of the molecule contains an anionic group, and

50 Z stands for the non-metallic atoms necessary to complete a 5- or 6-membered heterocyclic N-containing nucleus.

3. A direct-positive photographic element according to claim 2, wherein Q represents a group of the formula:



wherein:

65 each of R<sub>1</sub> and R<sub>4</sub> represents hydrogen, an alkyl group or an aryl group or R<sub>1</sub> together with R<sub>2</sub> represents the atoms necessary to complete a fused-on benzo ring.

4. A direct-positive photographic element according to claim 2, wherein the spectrally sensitizing dye corresponds to the formula:



X-

5



or  $L_5 = L_6$  wherein  $L_5$  and  $L_6$  are a methine group, and when  $n$  is 1, stands for a monovalent chemical bond.

5. A direct-positive photographic element according to claim 4, wherein the said substituent with Hammett constant of at least 0.30 is a nitro group, a cyano group, a carboxyl or sulpho group, an alkoxy carbonyl group, a carboxylic acyl group, a trifluoromethyl group, a cyanovinyl group, a fluorosulphonyl group, an alkylsulphonyl group, an alkylsulphinyl group, a trifluoromethoxy group, a trifluoromethylthio group, a carbamoyl or sulphamoyl group, or a  $-\text{SO}_2\text{NCO}$  alkyl group.

6. A direct-positive photographic element according to claim 1, wherein the emulsion layer also comprising a nitrobenzylidene or nitrostyryl desensitizing dye.

7. A direct-positive photographic element according to claim 1, wherein the silver halide grains are fogged by reduction sensitization in the presence of a compound of a metal more electropositive than silver.

8. A direct-positive photographic element according to claim 7, wherein said compound of a metal more electropositive than silver is a gold compound.

\* \* \* \* \*

wherein:

$Q$ ,  $L_1$ ,  $L_2$ ,  $L_3$ ,  $L_4$ ,  $m$ ,  $n$ ,  $R_5$  and  $X^-$  have the same significance as in claim 2,

$Y$  represents the atoms necessary to close a fused-on benzo or naphtho ring carrying one or more substituents at least one of which has a Hammett constant  $\sigma_P$  of at least 0.30, and

$Z_1$ , when  $n$  is 0, stands for oxygen, sulphur, selenium,

25

30

25

35

40

45

50

55

60

65